

# United States Patent

Bruengger et al.

[15] 3,647,466

[45] Mar. 7, 1972

[54] **PHOTOGRAPHIC MATERIAL FOR THE SILVER DYESTUFF BLEACHING PROCESS**

[72] Inventors: Heinrich Bruengger, Basel; Carlo Boragine, Fribourg, both of Switzerland

[73] Assignee: Ciba Limited, Basel, Switzerland

[22] Filed: Aug. 21, 1969

[21] Appl. No.: 852,083

[30] **Foreign Application Priority Data**

May 26, 1968 Switzerland ..... 12772/68

[52] U.S. Cl..... 96/99, 96/137

[51] Int. Cl..... G03c 1/10

[58] **Field of Search** ..... 96/109, 99

[56] **References Cited**

UNITED STATES PATENTS

2,503,776 4/1950 Sprague ..... 96/106 X

|           |         |                      |          |
|-----------|---------|----------------------|----------|
| 3,058,978 | 10/1962 | Berlin et al.....    | 96/106 X |
| 3,157,507 | 11/1964 | Bruengger et al..... | 96/99    |
| 3,255,012 | 6/1966  | Glockner et al. .... | 96/106 X |
| 3,348,949 | 10/1967 | Bannert et al. ....  | 96/106   |
| 3,354,170 | 11/1967 | Rosenoff.....        | 96/106 X |
| 3,410,848 | 11/1968 | Rauch et al. ....    | 96/106 X |

*Primary Examiner*—Norman G. Torchin

*Assistant Examiner*—John L. Goodrow

*Attorney*—Harry Goldsmith, Joseph G. Kolodny and Mario A. Monaco

[57] **ABSTRACT**

Photographic material for the silver dyestuff bleaching process is provided wherein at least one silver halide emulsion layer, containing a bleachable azo dyestuff as the image dyestuff also contains a benzelenazole-benzelenazole or benzelenazole-benzthiazole carbocyanine as red-sensitizer. This photographic material is characterized by an unexpectedly high relative sensitivity, especially in the presence of polyazo dyestuffs.

11 Claims, No Drawings

PHOTOGRAPHIC MATERIAL FOR THE SILVER  
DYESTUFF BLEACHING PROCESS

The present invention provides a photographic material for the silver dyestuff bleaching process wherein at least one silver halide emulsion layer, containing a bleachable azo dyestuff as the image dyestuff also contains a red-sensitizer of formula



optionally of betainelike structure, wherein A represents a hydrogen atom or an alkyl group containing 1 to 4 carbon atoms, B<sub>1</sub> and B<sub>2</sub> each represents an alkyl residue containing 1 to 4 carbon atoms, an alkylcarboxylic acid residue containing 1 to 5 carbon atoms, a sulphatoalkyl residue containing 1 to 4 carbon atoms or an alkylsulphonic acid residue, wherein alkyl represents a residue of formula —C<sub>n</sub>H<sub>2n</sub>— and n represents an integer having a value of 1 to 4, it also being possible for an acid group B<sub>1</sub> or B<sub>2</sub> to be present as a betainelike structure, R<sub>1</sub> and R<sub>2</sub> each represents an aromatic ring system containing at most two six-membered rings and fused-on in the manner indicated by the valency lines, Y<sup>-</sup> represents an anion, Z represents a sulphur or selenium atom and m is 1 in the case of a betainelike molecular structure and is 2 in the case of a non-betainelike molecular structure.

Betainelike structures results if at least one of the residues B<sub>1</sub> and B<sub>2</sub> represents a sulphatoalkyl residue or an alkylsulphonic acid residue or if B<sub>1</sub> and B<sub>2</sub> each represents an alkylcarboxylic acid residue. In the case of the betainelike structures the anion Y<sup>-</sup> is absent since the anion is already present in the molecule of the sensitizer itself, that is to say is bonded to the N-alkyl residue of the sensitizer by a homopolar bond. In this connection zwitter ions or internal salts may be mentioned. If the residues B<sub>1</sub> and B<sub>2</sub> each represents an alkyl residue or one of the two residues represents an alkyl residue and the other represents an alkyl-carboxylic acid residue, the sensitizers are of a nonbetainelike structure and the anion Y<sup>-</sup> neutralizes the positive charge of the actual sensitizer molecule.

If both B<sub>1</sub> and B<sub>2</sub> are alkyl residues, the dyestuffs are basic cyanine dyestuffs. If only one of the residues B<sub>1</sub> and B<sub>2</sub> represents an alkyl residue and the other represents an alkylsulphonic acid residue or sulphatoalkyl residue, the dyestuffs are neutral cyanine dyestuffs. Acid cyanine dyestuffs are present if B<sub>1</sub> and B<sub>2</sub> represent acid groups, that is to say carboxylic acid-alkyl, alkylsulphonic acid or sulphatoalkyl groups.

A photographic material for the silver dyestuff bleaching process which contains a red-sensitizer of formula



wherein A represents a hydrogen atom or an alkyl group containing 1 to 4 carbon atoms, B<sub>3</sub> represents an alkyl residue containing 1 to 4 carbon atoms or an alkylcarboxylic acid residue containing 1 to 5 carbon atoms, B<sub>4</sub> represents a sulphatoalkyl residue containing 1 to 4 carbon atoms or an alkylsulphonic acid residue, wherein alkyl represents a residue of formula —C<sub>n</sub>H<sub>2n</sub>— and n represents an integer having a

value of 1 to 4, preferably 1 to 3, B<sub>5</sub> represents an alkyl residue containing 1 to 4 carbon atoms, R<sub>1</sub> and R<sub>2</sub> each represents an aromatic ring system fused-on in the manner indicated by the valency lines, Y<sup>-</sup> represents an anion, Z represents a selenium or sulphur atom and m and p denote 1 or 2, is especially suitable.

A photographic material which contains a red-sensitizer of a nonbetainelike structure of formula



25 wherein A, B<sub>3</sub>, B<sub>5</sub>, R<sub>1</sub>, R<sub>2</sub>, Z, p and Y<sup>-</sup> have the meanings given above, is preferred.

The residue A in formulas (I) to (III) is in the so-called mesoposition of the trimethine chain of the molecule. A is either a hydrogen atom or a methyl, propyl, butyl or especially an ethyl residue.

The residues B<sub>1</sub> and B<sub>2</sub> in formula (I) are residues of formulas (IV) —alkylene-H, (V) —alkylene-COOH, (VI) —alkylene-O-SO<sub>3</sub>H or (VII) —alkylene-SO<sub>3</sub>H, wherein alkylene represents an alkylene residue containing 1 to 4 carbon atoms.

35 The following residues may be mentioned by way of examples: methyl, ethyl, propyl, isobutyl, acetic acid, propionic acid, valeric acid, sulphatomethyl, sulphatoethyl, propylsulphonic acid or butylsulphonic acid residues.

Sensitizers which are especially valuable are those of formula



55 wherein b<sub>6</sub> represents an ethyl, methylcarboxylic acid or ethylcarboxylic acid residue and A, R<sub>1</sub>, R<sub>2</sub>, Y<sup>-</sup>, Z and p have the meanings given above.

The residues R<sub>1</sub> and R<sub>2</sub> in formulas (I) to (III) and (VIII) represent ring systems which are fused-on in the manner indicated by the valency lines, which may be different from one another or identical. The residues R<sub>1</sub> and R<sub>2</sub> must exhibit an aromatic character and may contain at most two six-membered rings.

R<sub>1</sub> and R<sub>2</sub> may here represent the completion of, for example, the following residues: benzene or naphthalene residues, tetrahydronaphthalene residues or heterocyclic residues, for example, coumarone, thianaphthene or benzo- $\alpha$ -pyrane residues. All these residues can, of course, possess the most diverse substituents, such as, for example halogen atoms, alkyl, aryl or heterocyclic residues. Alkyl or aryl residues or heterocyclic residues can at the same time be bonded to the ring system either directly or via a heteroatom, for example, an oxygen or sulphur atom. Accordingly, further possibilities

for  $R_1$  and  $R_2$  are, for example, also diphenyl, furylbenzene or thiienylbenzene residues.

Red-sensitizers of formula



have proved very successful in the present use, in which formula  $R_3$  and  $R_4$  each represents a benzene or naphthalene residue which is fused-on in the manner indicated by the valency lines and is optionally substituted by halogen atoms or alkyl or alkoxy groups which each contain 1 to 3 carbon atoms, and  $A$ ,  $B_3$ ,  $B_5$ ,  $Y^-$ ,  $Z$  and  $p$  have the meanings given above.

Among such sensitizers, those of formula



are again preferred, wherein  $X_1$ ,  $X_2$ ,  $X_3$  and  $X_4$  each represents a hydrogen or halogen atom or an alkyl or alkoxy group each containing 1 to 3 carbon atoms, and  $A$ ,  $B_3$ ,  $B_5$ ,  $Y^-$ ,  $Z$  and  $p$  have the meanings given above.

Preferably, the residues  $X_1$  and  $X_3$  are respectively in the 6- or 7-position or in the 6'- or 7'-position and the residues  $X_2$  and  $X_4$  are respectively in the 5 and 5'-position.

At the same time, red-sensitizers of formula



wherein  $X_1$ ,  $X_2$ ,  $X_3$ ,  $X_4$ ,  $A$ ,  $B_3$ ,  $B_5$  and  $Y^-$ ,  $Z$  and  $p$  have the meanings given above are of especial interest.

Red-sensitizers of formula



10 wherein  $X_5$ ,  $X_6$ ,  $X_7$  and  $X_8$  each represents a hydrogen atom, a chlorine atom, a methyl, methoxy or ethoxy group and  $A$ ,  $B_3$ ,  $B_5$ ,  $Y^-$ ,  $Z$  and  $p$  have the meanings given above, have proved especially valuable.

15 The residue  $Y^-$  in formulas (I) to (III) and (VIII) to (XII) represents one of the usual anions used in the chemistry of the cyanine dyestuffs, these anions being known to be of minor importance for the sensitizing effect. (Compare F.M. Hamer "The Cyanine Dyes and Related Compounds," chapter 10, page 296). Sensitizers with preferred anions correspond to formula



wherein  $Y_1^-$  represents a halogen, thiocyanate, perchlorate, nitrate, methylsulphate, ethylsulphate or *p*-toluenesulphonate ion and  $A$ ,  $B_3$ ,  $B_5$ ,  $R_1$ ,  $R_2$ ,  $Z$  and  $p$  have the meanings given above.

Especially effective red-sensitizers correspond to formula (XIV)



wherein  $Y^-$ ,  $B_6$ ,  $X_5$ ,  $X_6$ ,  $X_7$ ,  $X_8$ ,  $Z$  and  $p$  have the meanings given above.

Suitable representatives of the red-sensitizers according to formula (I) are for example, the cyanine dyestuffs of Table I below, wherein the symbols represent the following:

I: Compound of formula No.  
II: Absorption maximum measured in ethanol in nm.  
III: Sensitization maximum measured in an exposed and developed gelatine-silver halide emulsion.

55 Page 15: \* Compound No. 55 additionally possesses an  $H_3C-$  group in the 7-position.

Page 15: \*\* Compound No. 56 possesses a fused-on benzene ring in the 6,7-position.

TABLE I



| I  | Z | $X_1$            | $X_2$            | $B_1$                                                                         | A                              | $B_2$                                   | $X_3$            | $X_4$             | $Y^-$                          | II  | III |
|----|---|------------------|------------------|-------------------------------------------------------------------------------|--------------------------------|-----------------------------------------|------------------|-------------------|--------------------------------|-----|-----|
| 1. | S | -H               | -Cl              | -C <sub>2</sub> H <sub>5</sub>                                                | -C <sub>2</sub> H <sub>5</sub> | -C <sub>2</sub> H <sub>5</sub>          | -H               | -OCH <sub>3</sub> | I <sup>-</sup>                 | 566 | 654 |
| 2. | S | -H               | -CH <sub>3</sub> | -C <sub>2</sub> H <sub>5</sub>                                                | -C <sub>2</sub> H <sub>5</sub> | -C <sub>2</sub> H <sub>5</sub>          | -H               | -CH <sub>3</sub>  | I <sup>-</sup>                 | 560 | 640 |
| 3. | S | -H               | -Cl              | -C <sub>2</sub> H <sub>5</sub>                                                | -C <sub>2</sub> H <sub>5</sub> | -CH <sub>2</sub> CH <sub>2</sub> -COOH  | -H               | -OCH <sub>3</sub> | I <sup>-</sup>                 | 564 | 640 |
| 4. | S | -H               | -CH <sub>3</sub> | -C <sub>2</sub> H <sub>5</sub>                                                | -C <sub>2</sub> H <sub>5</sub> | -CH <sub>2</sub> CH <sub>2</sub> -COOH  | -H               | -CH <sub>3</sub>  | I <sup>-</sup>                 | 560 | 650 |
| 5. | S | -CH <sub>3</sub> | -CH <sub>3</sub> | -C <sub>2</sub> H <sub>5</sub>                                                | -C <sub>2</sub> H <sub>5</sub> | -CH <sub>2</sub> CH <sub>2</sub> -COOH  | -H               | -CH <sub>3</sub>  | I <sup>-</sup>                 | 555 | 656 |
| 6. | S | -H               | -Cl              | -CH <sub>2</sub> CH <sub>2</sub> CH <sub>2</sub> SO <sub>3</sub> <sup>-</sup> | -C <sub>2</sub> H <sub>5</sub> | -C <sub>2</sub> H <sub>5</sub>          | -H               | -CH <sub>3</sub>  | -----                          | 565 | 656 |
| 7. | S | -CH <sub>3</sub> | -CH <sub>3</sub> | -CH <sub>2</sub> CH <sub>2</sub> CH <sub>2</sub> SO <sub>3</sub> <sup>-</sup> | -C <sub>2</sub> H <sub>5</sub> | -C <sub>2</sub> H <sub>5</sub>          | -H               | -CH <sub>3</sub>  | -----                          | 567 | 656 |
| 8. | S | -CH <sub>3</sub> | -CH <sub>3</sub> | -C <sub>2</sub> H <sub>5</sub>                                                | -C <sub>2</sub> H <sub>5</sub> | -C <sub>2</sub> H <sub>5</sub>          | -H               | -OCH <sub>3</sub> | -----                          | 565 | 600 |
| 9. | S | -H               | -H               | -C <sub>2</sub> H <sub>5</sub>                                                | -C <sub>2</sub> H <sub>5</sub> | -CH <sub>2</sub> -CH <sub>2</sub> -COOH | -CH <sub>3</sub> | -CH <sub>3</sub>  | -ClO <sub>4</sub> <sup>-</sup> | 561 | 640 |

TABLE I—Continued

| Z   | X <sub>1</sub> | X <sub>2</sub>                 | B <sub>1</sub>    | A                              | B <sub>2</sub>                                                                                    | X <sub>3</sub>                                                                   | X <sub>4</sub>                   | Y <sup>⊖</sup>                 | II             | III |     |
|-----|----------------|--------------------------------|-------------------|--------------------------------|---------------------------------------------------------------------------------------------------|----------------------------------------------------------------------------------|----------------------------------|--------------------------------|----------------|-----|-----|
| 10  | S              | -H                             | -Cl               | -C <sub>2</sub> H <sub>5</sub> | -C <sub>2</sub> H <sub>6</sub> —CH <sub>2</sub> —COOH                                             | -H                                                                               | -OCH <sub>3</sub>                | I <sup>-</sup>                 | 566            | 660 |     |
| 11  | S              | -H                             | -Cl               | -C <sub>2</sub> H <sub>5</sub> | -C <sub>2</sub> H <sub>5</sub>                                                                    | -H                                                                               | -CH <sub>3</sub>                 | I <sup>-</sup>                 | 560            | 650 |     |
| 12  | S              | -H                             | -Cl               | -C <sub>2</sub> H <sub>5</sub> | -C <sub>2</sub> H <sub>5</sub>                                                                    | -H                                                                               | -H                               | -ClO <sub>4</sub> <sup>-</sup> | 557            | 650 |     |
| 13  | S              | -H                             | -Cl               | -C <sub>2</sub> H <sub>5</sub> | -C <sub>2</sub> H <sub>5</sub>                                                                    | -H                                                                               | -H                               | I <sup>-</sup>                 | 558            | 650 |     |
| 14  | S              | -H                             | -Cl               | -C <sub>2</sub> H <sub>5</sub> | -C <sub>2</sub> H <sub>5</sub> —CH <sub>2</sub> —COOH                                             | -H                                                                               | -H                               | I <sup>-</sup>                 | 557            | 650 |     |
| 15  | S              | -H                             | -Cl               | -C <sub>2</sub> H <sub>5</sub> | -C <sub>2</sub> H <sub>5</sub> —CH <sub>2</sub> —COOH                                             | -H                                                                               | -H                               | -ClO <sub>4</sub> <sup>-</sup> | 557            | 654 |     |
| 16  | S              | -H                             | -Cl               | -C <sub>2</sub> H <sub>5</sub> | -C <sub>2</sub> H <sub>6</sub> —CH <sub>2</sub> —COOH                                             | -H                                                                               | -CH <sub>3</sub>                 | -ClO <sub>4</sub> <sup>-</sup> | 560            | 656 |     |
| 17  | S              | -CH <sub>3</sub>               | -CH <sub>3</sub>  | -C <sub>2</sub> H <sub>5</sub> | -C <sub>2</sub> H <sub>5</sub>                                                                    | -H                                                                               | -CH <sub>3</sub>                 | I <sup>-</sup>                 | 562            | 640 |     |
| 18  | S              | -H                             | -Cl               | -C <sub>2</sub> H <sub>5</sub> | -C <sub>2</sub> H <sub>5</sub>                                                                    | -CH <sub>3</sub>                                                                 | -CH <sub>3</sub>                 | I <sup>-</sup>                 | 562            | 640 |     |
| 19  | S              | -H                             | -H                | -C <sub>2</sub> H <sub>5</sub> | -C <sub>2</sub> H <sub>5</sub> —CH <sub>2</sub> —COOH                                             | -H                                                                               | -H                               | I <sup>-</sup>                 | 554            | 640 |     |
| 20  | S              | -H                             | -Cl               | -C <sub>2</sub> H <sub>5</sub> | -C <sub>2</sub> H <sub>5</sub> —CH <sub>2</sub> —COOH                                             | -CH <sub>3</sub>                                                                 | -CH <sub>3</sub>                 | I <sup>-</sup>                 | 562            | 650 |     |
| 21  | S              | -H                             | -H                | -C <sub>2</sub> H <sub>5</sub> | -C <sub>2</sub> H <sub>5</sub> —CH <sub>2</sub> —COOH                                             | -CH <sub>3</sub>                                                                 | -CH <sub>3</sub>                 | I <sup>-</sup>                 | 560            | 640 |     |
| 22  | S              | -H                             | -H                | -C <sub>2</sub> H <sub>5</sub> | -C <sub>2</sub> H <sub>5</sub> —CH <sub>2</sub> —COOH                                             | -H                                                                               | -CH <sub>3</sub>                 | I <sup>-</sup>                 | 557            | 644 |     |
| 23  | S              | -CH <sub>3</sub>               | -CH <sub>3</sub>  | -C <sub>2</sub> H <sub>5</sub> | -C <sub>2</sub> H <sub>5</sub> —CH <sub>2</sub> —COOH                                             | -H                                                                               | -OCH <sub>3</sub>                | I <sup>-</sup>                 | 567            | 650 |     |
| 24  | S              | -CH <sub>3</sub>               | -CH <sub>3</sub>  | -C <sub>2</sub> H <sub>5</sub> | -C <sub>2</sub> H <sub>5</sub> —CH <sub>2</sub> —COOH                                             | -H                                                                               | -H                               | I <sup>-</sup>                 | 560            | 640 |     |
| 25  | S              | -H                             | -CH <sub>3</sub>  | -C <sub>2</sub> H <sub>5</sub> | -C <sub>2</sub> H <sub>5</sub>                                                                    | -CH <sub>3</sub>                                                                 | -CH <sub>3</sub>                 | I <sup>-</sup>                 | 553            | 625 |     |
| 26  | S              | -H                             | -CH <sub>3</sub>  | -C <sub>2</sub> H <sub>5</sub> | -H                                                                                                | -CH <sub>3</sub>                                                                 | -CH <sub>3</sub>                 | I <sup>-</sup>                 | 563            | 640 |     |
| 27  | S              | -H                             | -CH <sub>3</sub>  | -C <sub>2</sub> H <sub>5</sub> | -C <sub>2</sub> H <sub>5</sub>                                                                    | -CH <sub>3</sub>                                                                 | -CH <sub>3</sub>                 | I <sup>-</sup>                 | 557            | 640 |     |
| 28  | S              | -H                             | -CH <sub>3</sub>  | -C <sub>2</sub> H <sub>5</sub> | -C <sub>2</sub> H <sub>5</sub> —CH <sub>2</sub> —COOH                                             | -H                                                                               | -CH <sub>3</sub>                 | I <sup>-</sup>                 | 558            | 640 |     |
| 29  | S              | -H                             | -CH <sub>3</sub>  | -C <sub>2</sub> H <sub>5</sub> | -C <sub>2</sub> H <sub>5</sub> —CH <sub>2</sub> —COOH                                             | -H                                                                               | -CH <sub>3</sub>                 | I <sup>-</sup>                 | 560            | 650 |     |
| 30  | S              | -H                             | -CH <sub>3</sub>  | -C <sub>2</sub> H <sub>5</sub> | -C <sub>2</sub> H <sub>5</sub> —CH <sub>2</sub> —COOH                                             | -H                                                                               | -CH <sub>3</sub>                 | I <sup>-</sup>                 | 559            | 650 |     |
| 31  | S              | -H                             | -Cl               | -C <sub>2</sub> H <sub>5</sub> | -C <sub>2</sub> H <sub>5</sub> —CH <sub>2</sub> —COOH                                             | -H                                                                               | -OCH <sub>3</sub>                | I <sup>-</sup>                 | 564            | 650 |     |
| 32  | S              | -H                             | -CH <sub>3</sub>  | -C <sub>2</sub> H <sub>5</sub> | -C <sub>2</sub> H <sub>5</sub> —CH <sub>2</sub> —COOH                                             | -H                                                                               | -CH <sub>3</sub>                 | I <sup>-</sup>                 | 559            | 650 |     |
| 33  | S              | -H                             | -CH <sub>3</sub>  | -C <sub>2</sub> H <sub>5</sub> | -C <sub>2</sub> H <sub>5</sub> —CH <sub>2</sub> —COOH                                             | -H                                                                               | -CH <sub>3</sub>                 | I <sup>-</sup>                 | 560            | 654 |     |
| 34  | S              | -H                             | -CH <sub>3</sub>  | -C <sub>2</sub> H <sub>5</sub> | -C <sub>2</sub> H <sub>5</sub> —CH <sub>2</sub> —SO <sub>3</sub> <sup>-</sup>                     | -H                                                                               | -H                               | I <sup>-</sup>                 | 563            | 640 |     |
| 35  | S              | -CH <sub>3</sub>               | -CH <sub>3</sub>  | -C <sub>2</sub> H <sub>5</sub> | -CH <sub>2</sub> —CH <sub>2</sub> —SO <sub>3</sub> <sup>-</sup>                                   | -H                                                                               | -CH <sub>3</sub>                 | I <sup>-</sup>                 | 560            | 646 |     |
| 36  | S              | -CH <sub>3</sub>               | -H                | -C <sub>2</sub> H <sub>5</sub> | -CH <sub>2</sub> —CH <sub>2</sub> —COOH                                                           | -H                                                                               | -H                               | I <sup>-</sup>                 | 557            | 650 |     |
| 37  | S              | -H                             | -Cl               | -C <sub>2</sub> H <sub>5</sub> | -CH <sub>2</sub> —CH <sub>2</sub> —COOH                                                           | -H                                                                               | -H                               | I <sup>-</sup>                 | 556            | 640 |     |
| 38  | S              | -H                             | -H                | -C <sub>2</sub> H <sub>5</sub> | -CH <sub>2</sub> —CH <sub>2</sub> —CH <sub>2</sub> —SO <sub>3</sub> <sup>-</sup>                  | -H                                                                               | -CH <sub>3</sub>                 | I <sup>-</sup>                 | 563            | 660 |     |
| 39  | S              | -OCH <sub>3</sub>              | -H                | -C <sub>2</sub> H <sub>5</sub> | -CH <sub>2</sub> —CH <sub>2</sub> —COOH                                                           | -H                                                                               | -CH <sub>3</sub>                 | I <sup>-</sup>                 | 560            | 650 |     |
| 40  | S              | -H                             | -CH <sub>3</sub>  | -C <sub>2</sub> H <sub>5</sub> | -CH <sub>2</sub> —CH <sub>2</sub> —COOH                                                           | -H                                                                               | -H                               | I <sup>-</sup>                 | 555            | 650 |     |
| 41  | S              | -H                             | -CH <sub>3</sub>  | -C <sub>2</sub> H <sub>5</sub> | -CH <sub>2</sub> —CH <sub>2</sub> —COOH                                                           | -H                                                                               | -H                               | I <sup>-</sup>                 | 554            | 640 |     |
| 42  | S              | -H                             | -H                | -C <sub>2</sub> H <sub>5</sub> | -C <sub>2</sub> H <sub>5</sub>                                                                    | -H                                                                               | -H                               | I <sup>-</sup>                 | 560            | 650 |     |
| 43  | S              | -H                             | -Cl               | -C <sub>2</sub> H <sub>5</sub> | -CH <sub>2</sub> —CH <sub>2</sub> —CH <sub>2</sub> —SO <sub>3</sub> <sup>-</sup>                  | -H                                                                               | -H                               | I <sup>-</sup>                 | 560            | 650 |     |
| 44  | S              | -CH <sub>3</sub>               | -CH <sub>3</sub>  | -C <sub>2</sub> H <sub>5</sub> | -CH <sub>2</sub> —CH <sub>2</sub> —COOH                                                           | -C <sub>2</sub> H <sub>5</sub>                                                   | -CH <sub>3</sub>                 | I <sup>-</sup>                 | 560            | 650 |     |
| 45  | S              | -H                             | -Cl               | -C <sub>2</sub> H <sub>5</sub> | -CH <sub>2</sub> —CH <sub>2</sub> —CH <sub>2</sub> —CH <sub>2</sub> —SO <sub>3</sub> <sup>-</sup> | -H                                                                               | -CH <sub>3</sub>                 | I <sup>-</sup>                 | 560            | 654 |     |
| 46  | S              | -CH <sub>3</sub>               | -H                | -C <sub>2</sub> H <sub>5</sub> | -CH <sub>2</sub> —CH <sub>2</sub> —COOH                                                           | -C <sub>2</sub> H <sub>5</sub>                                                   | -CH <sub>3</sub>                 | I <sup>-</sup>                 | 555            | 640 |     |
| 47  | S              | -C <sub>2</sub> H <sub>5</sub> | -H                | -C <sub>2</sub> H <sub>5</sub> | -CH <sub>2</sub> —CH <sub>2</sub> —COOH                                                           | -C <sub>2</sub> H <sub>5</sub>                                                   | -CH <sub>3</sub>                 | I <sup>-</sup>                 | 559            | 640 |     |
| 48  | S              | -H                             | -CH <sub>3</sub>  | -C <sub>2</sub> H <sub>5</sub> | -CH <sub>2</sub> —CH <sub>2</sub> —COOH                                                           | -C <sub>2</sub> H <sub>5</sub>                                                   | -CH <sub>3</sub>                 | I <sup>-</sup>                 | 562            | 660 |     |
| 49  | S              | -OCH <sub>3</sub>              | -H                | -C <sub>2</sub> H <sub>5</sub> | -CH <sub>2</sub> —CH <sub>2</sub> —COOH                                                           | -C <sub>2</sub> H <sub>5</sub>                                                   | -CH <sub>3</sub>                 | I <sup>-</sup>                 | 560            | 644 |     |
| 50  | S              | -H                             | -H                | -C <sub>2</sub> H <sub>5</sub> | -CH <sub>2</sub> —CH <sub>2</sub> —CH <sub>2</sub> —SO <sub>3</sub> <sup>-</sup>                  | -C <sub>2</sub> H <sub>5</sub>                                                   | -CH <sub>3</sub>                 | I <sup>-</sup>                 | 558            | 650 |     |
| 51  | S              | -H                             | -Br               | -C <sub>2</sub> H <sub>5</sub> | -CH <sub>2</sub> —CH <sub>2</sub> —COOH                                                           | -C <sub>2</sub> H <sub>5</sub>                                                   | -CH <sub>3</sub>                 | I <sup>-</sup>                 | 558            | 660 |     |
| 52  | S              | -H                             | -H                | -C <sub>2</sub> H <sub>5</sub> | -CH <sub>2</sub> —CH <sub>2</sub> —CH <sub>2</sub> —SO <sub>3</sub> <sup>-</sup>                  | -C <sub>2</sub> H <sub>5</sub>                                                   | -CH <sub>3</sub>                 | I <sup>-</sup>                 | 558            | 646 |     |
| 53  | S              | -H                             | -Cl               | -C <sub>2</sub> H <sub>5</sub> | -CH <sub>2</sub> —COOH                                                                            | -C <sub>2</sub> H <sub>5</sub>                                                   | -CH <sub>3</sub>                 | I <sup>-</sup>                 | 550            | 640 |     |
| 54  | S              | -CH <sub>3</sub>               | -CH <sub>3</sub>  | -C <sub>2</sub> H <sub>5</sub> | -CH <sub>2</sub> —CH <sub>2</sub> —COOH                                                           | -C <sub>2</sub> H <sub>5</sub>                                                   | -CH <sub>3</sub>                 | I <sup>-</sup>                 | 560            | 640 |     |
| 55  | S              | -H                             | -H                | -C <sub>2</sub> H <sub>5</sub> | -CH <sub>2</sub> —CH <sub>2</sub> —COOH                                                           | -C <sub>2</sub> H <sub>5</sub>                                                   | -CH <sub>3</sub>                 | I <sup>-</sup>                 | 555            | 640 |     |
| 56* | S              | (**)                           | -H                | -C <sub>2</sub> H <sub>5</sub> | -CH <sub>2</sub> —CH <sub>2</sub> —COOH                                                           | -C <sub>2</sub> H <sub>5</sub>                                                   | -CH <sub>3</sub>                 | I <sup>-</sup>                 | 570            | 660 |     |
| 57  | S              | -H                             | -H                | -C <sub>2</sub> H <sub>5</sub> | -CH <sub>2</sub> —CH <sub>2</sub> —O—SO <sub>3</sub> <sup>-</sup>                                 | -C <sub>2</sub> H <sub>5</sub>                                                   | -CH <sub>3</sub>                 | I <sup>-</sup>                 | 560            | 650 |     |
| 58  | S              | -CH <sub>3</sub>               | -CH <sub>3</sub>  | -C <sub>2</sub> H <sub>5</sub> | -CH <sub>2</sub> —CH <sub>2</sub> —CH <sub>2</sub> —SO <sub>3</sub> <sup>-</sup>                  | -C <sub>2</sub> H <sub>5</sub>                                                   | -CH <sub>3</sub>                 | I <sup>-</sup>                 | 563            | 650 |     |
| 59  | S              | -Cl                            | -H                | -C <sub>2</sub> H <sub>5</sub> | -CH <sub>2</sub> —CH <sub>2</sub> —COOH                                                           | -C <sub>2</sub> H <sub>5</sub>                                                   | -CH <sub>3</sub>                 | I <sup>-</sup>                 | 665            | 665 |     |
| 60  | S              | -H                             | -CH <sub>3</sub>  | -C <sub>2</sub> H <sub>5</sub> | -CH <sub>2</sub> —CH <sub>2</sub> —CH <sub>2</sub> —SO <sub>3</sub> <sup>-</sup>                  | -C <sub>2</sub> H <sub>5</sub>                                                   | -O—C <sub>2</sub> H <sub>5</sub> | I <sup>-</sup>                 | 569            | 655 |     |
| 61  | S              | -H                             | -OCH <sub>3</sub> | -C <sub>2</sub> H <sub>5</sub> | -C <sub>2</sub> H <sub>5</sub>                                                                    | -CH <sub>2</sub> —CH <sub>2</sub> —CH <sub>2</sub> —SO <sub>3</sub> <sup>-</sup> | -H                               | -OCH <sub>3</sub>              | I <sup>-</sup> | 568 | 655 |
|     |                |                                |                   |                                |                                                                                                   |                                                                                  |                                  |                                | F299-30        | 0   |     |
| 62  | S              | -H                             | -CH <sub>3</sub>  | -C <sub>2</sub> H <sub>5</sub> | -CH <sub>2</sub> —CH <sub>2</sub> —CH <sub>2</sub> —SO <sub>3</sub> <sup>-</sup>                  | -C <sub>2</sub> H <sub>5</sub>                                                   | -CH <sub>3</sub>                 | I <sup>-</sup>                 | 562            | 660 |     |
| 63  | S              | -H                             | -OCH <sub>3</sub> | -C <sub>2</sub> H <sub>5</sub> | -CH <sub>2</sub> —CH <sub>2</sub> —CH <sub>2</sub> —SO <sub>3</sub> <sup>-</sup>                  | -C <sub>2</sub> H <sub>5</sub>                                                   | -CH <sub>3</sub>                 | I <sup>-</sup>                 | 576            | 660 |     |
| 64  | S              | -H                             | -Br               | -C <sub>2</sub> H <sub>5</sub> | -CH <sub>2</sub> —CH <sub>2</sub> —CH <sub>2</sub> —SO <sub>3</sub> <sup>-</sup>                  | -C <sub>2</sub> H <sub>5</sub>                                                   | -CH <sub>3</sub>                 | I <sup>-</sup>                 | 566            | 660 |     |
| 65  | S              | -H                             | -Br               | -C <sub>2</sub> H <sub>5</sub> | -CH <sub>2</sub> —CH <sub>2</sub> —CH <sub>2</sub> —SO <sub>3</sub> <sup>-</sup>                  | -C <sub>2</sub> H <sub>5</sub>                                                   | -Br                              | I <sup>-</sup>                 | 567            | 655 |     |
| 66  | Se             | -H                             | -CH <sub>3</sub>  | -C <sub>2</sub> H <sub>5</sub> | -H                                                                                                | -C <sub>2</sub> H <sub>5</sub>                                                   | -CH <sub>3</sub>                 | I <sup>-</sup>                 | 580            | 620 |     |
| 67  | Se             | -H                             | -H                | -C <sub>2</sub> H <sub>5</sub> | -C <sub>2</sub> H <sub>5</sub>                                                                    | -H                                                                               | -OCH <sub>3</sub>                | I <sup>-</sup>                 | 567            | 620 |     |
| 68  | Se             | -H                             | -CH <sub>3</sub>  | -C <sub>2</sub> H <sub>5</sub> | -H                                                                                                | -C <sub>2</sub> H <sub>5</sub>                                                   | -CH <sub>3</sub>                 | I <sup>-</sup>                 | 587            | 630 |     |
| 69  | Se             | -H                             | -H                | -C <sub>2</sub> H <sub>5</sub> | -C <sub>2</sub> H <sub>5</sub>                                                                    | -C <sub>2</sub> H <sub>5</sub>                                                   | -H                               | I <sup>-</sup>                 | 562            | 650 |     |
| 70  | Se             | -H                             | -H                | -C <sub>2</sub> H <sub>5</sub> | -C <sub>2</sub> H <sub>5</sub>                                                                    | -C <sub>2</sub> H <sub>5</sub>                                                   | -H                               | I <sup>-</sup>                 | 560            | 654 |     |
| 71  | Se             | -H                             | -H                | -C <sub>2</sub> H <sub>5</sub> | -C <sub>2</sub> H <sub>5</sub>                                                                    | -C <sub>2</sub> H <sub>5</sub>                                                   | -CH <sub>3</sub>                 | I <sup>-</sup>                 | 563            | 660 |     |
| 72  | Se             | -H                             | -H                | -C <sub>2</sub> H <sub>5</sub> | -C <sub>2</sub> H <sub>5</sub>                                                                    | -C <sub>2</sub> H <sub>5</sub>                                                   | -OCH <sub>3</sub>                | I <sup>-</sup>                 | 567            | 650 |     |
| 73  | Se             | -CH <sub>3</sub>               | -CH <sub>3</sub>  | -C <sub>2</sub> H <sub>5</sub> | -H                                                                                                | -C <sub>2</sub> H <sub>5</sub>                                                   | -CH <sub>3</sub>                 | I <sup>-</sup>                 | 587            | 626 |     |

TABLE I—Continued

| I  | Z  | X <sub>1</sub>   | X <sub>2</sub>    | B <sub>1</sub>                                     | A                              | B <sub>2</sub>                                     | X <sub>3</sub>   | X <sub>4</sub>                          | Y <sup>⊖</sup>  | II  | III |
|----|----|------------------|-------------------|----------------------------------------------------|--------------------------------|----------------------------------------------------|------------------|-----------------------------------------|-----------------|-----|-----|
| 74 | Se | —H               | —OCH <sub>3</sub> | —C <sub>2</sub> H <sub>5</sub>                     | —H                             | —C <sub>2</sub> H <sub>5</sub>                     | —H               | —OCH <sub>3</sub>                       | I <sup>⊖</sup>  | 593 | 636 |
| 75 | Se | —H               | —CH <sub>3</sub>  | —C <sub>2</sub> H <sub>5</sub>                     | —H                             | —C <sub>2</sub> H <sub>5</sub>                     | —H               | —CH <sub>3</sub>                        | Br <sup>⊖</sup> | 580 | 624 |
| 76 | Se | —H               | —H                | —C <sub>2</sub> H <sub>5</sub>                     | —H                             | —C <sub>2</sub> H <sub>5</sub>                     | —H               | —OCH <sub>3</sub>                       | I <sup>⊖</sup>  | 584 | 624 |
| 77 | Se | —H               | —OCH <sub>3</sub> | —C <sub>2</sub> H <sub>5</sub>                     | —H                             | —C <sub>2</sub> H <sub>5</sub>                     | —CH <sub>3</sub> | —CH <sub>3</sub>                        | I <sup>⊖</sup>  | 590 | 630 |
| 78 | Se | —H               | —H                | —C <sub>2</sub> H <sub>5</sub>                     | —C <sub>2</sub> H <sub>5</sub> | —CH <sub>2</sub> —CH <sub>2</sub> —COOH            | —CH <sub>3</sub> | —CH <sub>3</sub>                        | I <sup>⊖</sup>  | 564 | 610 |
| 79 | Se | —H               | —CH <sub>3</sub>  | —C <sub>2</sub> H <sub>5</sub>                     | —C <sub>2</sub> H <sub>5</sub> | —C <sub>2</sub> H <sub>5</sub>                     | —H               | —CH <sub>3</sub>                        | I <sup>⊖</sup>  | 563 | 650 |
| 80 | Se | —H               | —H                | —CH <sub>2</sub> —CH <sub>2</sub> —COOH            | —C <sub>2</sub> H <sub>5</sub> | —C <sub>2</sub> H <sub>5</sub>                     | —H               | —CH <sub>2</sub> —CH <sub>2</sub> —COOH | I <sup>⊖</sup>  | 561 | 660 |
| 81 | Se | —H               | —CH <sub>3</sub>  | —C <sub>2</sub> H <sub>5</sub>                     | —C <sub>2</sub> H <sub>5</sub> | —C <sub>2</sub> H <sub>5</sub>                     | —H               | —OCH <sub>3</sub>                       | I <sup>⊖</sup>  | 569 | 660 |
| 82 | Se | —H               | —CH <sub>3</sub>  | —C <sub>2</sub> H <sub>5</sub>                     | —C <sub>2</sub> H <sub>5</sub> | —CH <sub>3</sub> —CH <sub>2</sub> —COOH            | —H               | —CH <sub>3</sub>                        | I <sup>⊖</sup>  | 565 | 660 |
| 83 | Se | —H               | —CH <sub>3</sub>  | —C <sub>2</sub> H <sub>5</sub>                     | —C <sub>2</sub> H <sub>5</sub> | —CH <sub>2</sub> —CH <sub>2</sub> —COOH            | —H               | —OCH <sub>3</sub>                       | I <sup>⊖</sup>  | 568 | 660 |
| 84 | Se | —H               | —CH <sub>3</sub>  | —C <sub>2</sub> H <sub>5</sub>                     | —C <sub>2</sub> H <sub>5</sub> | —CH <sub>2</sub> —CH <sub>2</sub> —COOH            | —CH <sub>3</sub> | —CH <sub>3</sub>                        | I <sup>⊖</sup>  | 565 | 660 |
| 85 | Se | —H               | —CH <sub>3</sub>  | —CH <sub>2</sub> —CH <sub>2</sub> —CH <sub>2</sub> | —C <sub>2</sub> H <sub>5</sub> | —C <sub>2</sub> H <sub>5</sub>                     | —H               | —CH <sub>3</sub>                        | -----           | 569 | 664 |
|    |    |                  |                   |                                                    | S O <sub>3</sub> <sup>—</sup>  |                                                    |                  |                                         |                 |     |     |
| 86 | Se | —H               | —CH <sub>3</sub>  | —C <sub>2</sub> H <sub>5</sub>                     | —C <sub>2</sub> H <sub>5</sub> | —CH <sub>2</sub> —CH <sub>2</sub> —CH <sub>2</sub> | —H               | —OCH <sub>2</sub> H <sub>5</sub>        | -----           | 575 | 665 |
|    |    |                  |                   |                                                    | S O <sub>3</sub> <sup>—</sup>  |                                                    |                  |                                         |                 |     |     |
| 87 | Se | —CH <sub>3</sub> | —CH <sub>3</sub>  | —CH <sub>2</sub> —CH <sub>2</sub> —CH <sub>2</sub> | —C <sub>2</sub> H <sub>5</sub> | —CH <sub>2</sub> —CH <sub>2</sub> —CH <sub>2</sub> | —CH <sub>3</sub> | —CH <sub>3</sub>                        | -----           | 570 | 660 |
|    |    |                  |                   |                                                    | S O <sub>3</sub> <sup>—</sup>  |                                                    |                  |                                         |                 |     |     |
| 88 | Se | —H               | —CH <sub>3</sub>  | —CH <sub>2</sub> —CH <sub>2</sub> —CH <sub>2</sub> | —C <sub>2</sub> H <sub>5</sub> | —C <sub>2</sub> H <sub>5</sub>                     | —CH <sub>3</sub> | —CH <sub>3</sub>                        | -----           | 571 | 665 |
|    |    |                  |                   |                                                    | S O <sub>3</sub> <sup>—</sup>  |                                                    |                  |                                         |                 |     |     |
| 89 | Se | —H               | —OCH <sub>3</sub> | —CH <sub>2</sub> —CH <sub>2</sub> —CH <sub>2</sub> | —C <sub>2</sub> H <sub>5</sub> | —C <sub>2</sub> H <sub>5</sub>                     | —CH <sub>3</sub> | —CH <sub>3</sub>                        | -----           | 577 | 670 |
|    |    |                  |                   |                                                    | S O <sub>3</sub> <sup>—</sup>  |                                                    |                  |                                         |                 |     |     |

Especially suitable representatives of the red-sensitizers of formula (I) are the compounds of formulas (I), (2), (16), 35 (40), (51), (53), (56), (66), (68) and more especially the compounds of formulas (5), (6), (45), (70), (71), (83) and (85). It follows from this that compounds which possess an ethyl group on one nitrogen atom, a propylsulphonic acid residue or propionic acid residue on the other nitrogen atom, 40 an ethyl group in the mesoposition and chlorine atoms, methyl groups or methoxy groups as substituents in the nuclei are especially effective sensitizers in photographic material for the silver dyestuff bleaching process.

The cyanine dyestuffs which according to the invention are 45 to be used as red-sensitizers in photographic material for the silver color bleaching process are in part known or can be manufactured according to known methods which are for example, described in the book by F. M. Hamer "The Cyanine Dyes and Related Compounds," chapters V and VI (Interscience Publishers New York 1964). Further manufacturing processes are, inter alia, also described in German Patent Nos. 917,330 and 929,080, French Pat. No. 1,166,246, Belgian Pat. No. 571,034 and U.S. Pat. No. 2,503,776.

A suitable method for the manufacture of the sensitizers of 55 formula (I) for example, comprises condensing a quaternary cyclammonium salt of formula



with a compound of formula



or condensing a compound of formula



or



with a compound of formula



wherein A, B<sub>1</sub>, B<sub>2</sub>, R<sub>1</sub>, R<sub>2</sub>, Y<sup>⊖</sup> and n have the meanings given above.

Red-sensitizers of formula (I) which contain acid groups which do not participate in a betainelike structure may be 70 present as free acids or as salts, especially as alkali salts such as, for example, sodium or potassium salts.

In the silver dyestuff bleaching process an increase in the sensitivity of the individual layers is especially important if the light-sensitive silver halide layer, when being exposed, already 75 contains a dyestuff which reduces the effective sensitivity of

the layer through absorption of the exposure light. The sensitization of such layers containing dyestuff is now rendered considerably more difficult by the fact that the dyestuffs incorporated into the layer, in addition to this sensitivity-reducing effect of the absorption, possess a strong desensitizing effect on the emulsion.

According to the invention unexpectedly high relative sensitivities are now achieved in sensitizing photographic layers for the silver dyestuff bleaching process if a cyanine dyestuff of formula (I) is added as a red-sensitizer to the silver salt emulsions containing the azo dyestuff.

Especially valuable substances are red-sensitizers of formula (I) which are capable of forming the J-bands. They are distinguished by a very characteristic sensitization band with a steep drop towards the longer wavelengths and show a sensitization maximum which is bathochromically displaced by 70 to 120 nm. relative to the absorption maximum in alcoholic solution. This formation of a polymerization band, the so-called J-band, described as a second-order sensitization, is technically valuable not only as regards the position of the sensitization maximum but also as a result of the relative sensitivities thereby achieved.

The red-sensitizers to be used according to the invention in photographic material for the silver dyestuff bleaching process have already been used as sensitizers in gelatine emulsions containing color coupling agents. These gelatine emulsions containing color coupling agents were used for the production of colored photographic images according to the chromogenic development principle. In such layers these sensitizers were distinguished by the fact that their sensitizing effect was unchanged, or at most slightly changed, by the presence of the color coupling agent. Nevertheless the fact that such sensitizers can also be successfully used in layers containing azo dyestuff for the silver dyestuff bleaching process was unforeseeable and surprising. Thus it is known that azo dyestuffs are in general more substantive in dyeing than is the case for the colorless components used as coupling agents. This is especially true of polyazo dyestuffs (which includes substantially all cyanazo dyestuffs) which reduce the sensitizing effect of the hitherto usual sensitizers. It was, therefore, to be expected that in the case of the layers of a silver dyestuff bleaching material containing azo dyestuffs an adequate sensitizing effect of the sensitizer on the silver halide would not be achieved or that such an effect would be entirely prevented. Thus it was to be assumed that the azo dyestuff would be able to displace the sensitizer adsorbed on the silver halides or that the dyestuff would form an inactive compound with the sensitizer. The extraordinarily great improvement in the sensitivity achieved with the red sensitizers used in accordance with the invention in the presence of azo dyestuffs, especially polyazo dyestuffs, was thus completely unexpected.

It is furthermore known that azo dyestuffs are desensitizers and reduce the sensitivity achievable by ordinary cyanine sensitizers.

The high sensitivity attainable by the red-sensitizers used in accordance with the invention is also achieved in layers with azo dyestuffs which are fixed by precipitation with basic precipitants, such as, for example biguanides. This is surprising because these basic precipitants (biguanides) are known to act as desensitizers and therefore their presence in the emulsion would according to all expectations have to have an unfavorable effect on the sensitization.

Equally, especially good results are achieved when using azo dyestuffs containing phenol groups. Here it has been known for a long time that azo dyestuffs containing phenol groups interfere with the effect of the known sensitizers.

The present sensitizers can be employed independently of the nature of the silver halide used. Alongside gelatine, other colloids can also be used as layer-forming agents. The present sensitizers can furthermore not only be used in multilayer material but can, for example, also be employed in mixed grain emulsions. The emulsions can furthermore contain casting additives of various kinds, for example wetting agents, hardeners or stabilizers.

Usually, the red-sensitizers of formula (I) are used in a layer containing a bluish-green bleachable azo dyestuff.

The following examples illustrate the invention. The percentages in the examples are percentages by weight.

#### EXAMPLE 1

Various ethanolic solutions of sensitizers are added, in each case to equal parts of a silver bromide-iodide emulsion containing 53 g. of silver and 70 g. of gelatine per 1 kg. of emulsion, at 40° C., so that a sensitizer concentration of 220 mg./mol of silver results.

|    | Emulsion | Sensitizer of Formula |
|----|----------|-----------------------|
| 15 |          |                       |
|    | A        | (1)                   |
|    | B        | (2)                   |
|    | C        | (3)                   |
|    | D        | (5)                   |
| 20 | E        | (6)                   |

For comparison purposes, emulsions F and G are additionally manufactured, containing so-called symmetrical sensitizers which differ from the sensitizers according to the invention:



(XXI)



Subsequently, in addition to the usual additives such as stabilizer, wetting agent, plasticizer and hardener, an aqueous solution of the bluish-green dyestuff of formula (XXII) is added to emulsions A to G, and in an amount which produces a dyestuff concentration of 13 g./kg. of emulsion.

(XXII)



Solutions A to G are cast on a transparent film substrate with a silver application of 3 g./m<sup>2</sup>. The cast layers are exposed sensitometrically behind a grey wedge with a yellow filter, and thereafter the material is developed as follows:

1. 6 Minutes development in a bath which per liter of water contains 50 g. of anhydrous sodium sulphite, 0.2 g. of 1-phenyl-3-pyrazolidone, 6 g. of hydroquinone, 35 g. of anhydrous sodium carbonate, 4 g. of potassium bromide and 0.3 g. of benztriazole;
2. 5 minutes soaking, 6 minutes fixing in a solution of 200 g. of crystalline sodium thiosulphate and 20 g. of potassium metabisulphite in 1 liter of water, and again 5 minutes soaking;
3. 2 to 12 minutes dyestuff bleaching with a solution which per

liter of water contains 50 to 80 g. of potassium bromide, 40 to 80 g. of thiourea, 35 to 80 g. of 30 percent strength sulphuric acid and 0.01 and 2-amino-3-oxyphenazine;

4. 10 minutes soaking and 5 minutes bleaching of residual silver with a solution of 60 g. of crystalline copper sulphate, 80 g. of potassium bromide and 15 ml. of 30 percent strength hydrochloric acid per liter of water;

5. soaking, fixing and soaking as indicated under 2.

The unexposed cast films A to E are also spectrally exposed to light in a spectrosensitometer. The material is processed as previously indicated under items 1 and 2, that is to say only a black and white development is carried out.

The results are summarized in the table below. The lower value of the relative sensitivity  $\log E$  represents higher sensitivity.

| Emulsion | Sensitization Maximum in nm | Spectrum                        | Color Development<br>Relative Sensitivity<br>$\log E$ |
|----------|-----------------------------|---------------------------------|-------------------------------------------------------|
| A        | 660                         |                                 | 2.98                                                  |
| B        | 656                         |                                 | 2.83                                                  |
| C        | 640                         |                                 | 3.09                                                  |
| D        | 652                         |                                 | 1.78                                                  |
| E        | 658                         |                                 | 1.14                                                  |
| F        | 560                         | weak image, cannot be evaluated |                                                       |
| G        | 560                         |                                 | 3.62                                                  |

The sensitizers used according to the invention in emulsions A to E produce a higher sensitivity and result in a sensitization maximum which is displaced to longer wavelengths than the sensitizers in emulsions F and G employed for comparison.

For a red-sensitive emulsion in a color reproduction material, sensitization with a maximum of 600 nm. and above is generally required, preferably at 640 to 700 nm.

5

plying 1.8 g./m.<sup>2</sup> of silver. The cast films are exposed and processed as indicated in Example 1. The results are summarized in the table below.

| Emulsion | Sensitization Maximum in nm | Spectrum | Color Development<br>Relative Sensitivity<br>$\log E$ |
|----------|-----------------------------|----------|-------------------------------------------------------|
| A        | 655                         |          | 3.43                                                  |
| B        | 600                         |          | 3.70                                                  |
| C        | 645                         |          | 3.00                                                  |
| D        | 650                         |          | 2.66                                                  |
| E        | 570                         |          | 4.00                                                  |

15

The sensitizers used according to the invention are emulsions A to D produce a higher sensitivity and result in a sensitization maximum which is displaced to longer wavelengths than the sensitizers in emulsion E employed for comparison purposes.

### EXAMPLE 3

25 The procedure described in Example 2 is adopted. The following are used as sensitizers according to the invention:

| Emulsion | Sensitizers of Formula |
|----------|------------------------|
| A        | (1)                    |
| B        | (5)                    |
| C        | (6)                    |

30 35 For comparison purposes, emulsion D is additionally manufactured, containing a so-called symmetrical sensitizer of formula (XX) which differs from the sensitizers according to the invention.

40 The compound of formula



### EXAMPLE 2

Various ethanol solutions of sensitizers are added in each case to equal parts of a silver bromide-iodide emulsion containing 21 g. of silver and 90 g. of gelatine per 1 kg. of emulsion, at 40° C., so that a sensitizer concentration of 200 mg./mol of silver results.

55 is used as a bluish-green image dyestuff. The results are summarized in the table below.

| Emulsion | Sensitization Maximum in nm | Spectrum | Color Development<br>Relative Sensitivity<br>$\log E$ |
|----------|-----------------------------|----------|-------------------------------------------------------|
| A        | 652                         |          | 3.81                                                  |
| B        | 650                         |          | 3.00                                                  |
| C        | 650                         |          | 2.72                                                  |
| D        | 570                         |          | 4.04                                                  |

60 65 The sensitizers used according to the invention in emulsions A to C produce a higher sensitivity and result in a sensitization maximum which is displaced to longer wavelengths than the sensitizers in emulsion D employed for comparison purposes.

### EXAMPLE 4

70 The procedure in Example 2 is adopted. The compound of formula (6) is used as a sensitizer according to the invention in emulsion A. For comparison, emulsion B is manufactured, containing the so-called symmetrical sensitizer of formula (XX). The compound of formula

For comparison, emulsion E is also manufactured, containing a so-called symmetrical sensitizer of formula (XX) which differs from the sensitizers according to the invention.

Subsequently, an aqueous solution of the bluish-green dyestuff of formula (XXII) is added to emulsions A to E in addition to the usual additives, for example, stabilizers, wetting agents, plasticizers and hardeners, in an amount which results in a dyestuff concentration of 4 g./kg. of emulsion.

Solutions A to G are cast on a white-opaque substrate, ap-



is used as the bluish-green image dyestuff. The results are summarized in the table below.

| Emulsion | Sensitization Maximum in nm | Color Development Relative Sensitivity log E |
|----------|-----------------------------|----------------------------------------------|
| A        | 650                         | 2.83                                         |
| B        | 570                         | 3.41                                         |

The sensitizer used according to the invention in emulsion A produces a higher sensitivity and results in a sensitization maximum which is displaced to longer wavelengths than the symmetrical sensitizer of emulsion B.

#### EXAMPLE 5

Various ethanol solutions of sensitizers are added in each case to equal parts of a silver bromide-iodide emulsion containing 53 g. of silver and 70 g. of gelatine per 1 kg. of emulsion, at 40° C., so that a sensitizer concentration of 160 mg./mol of silver results:

| Emulsion | Sensitizer of Formula |
|----------|-----------------------|
| A        | (66)                  |
| B        | (67)                  |
| C        | (68)                  |
| D        | (70)                  |
| E        | (71)                  |

For comparison, emulsions F and G are additionally manufactured, containing so-called symmetrical sensitizers which differ from the sensitizers according to the invention.

Emulsion F: Sensitizer of formula (XX)

Emulsion G: Sensitizer of formula (XXI)

Subsequently, an aqueous solution of the bluish-green dyestuff of formula (XXII) is added to emulsions A to G in addition to the usual additives, for example stabilizer, wetting agent, plasticizer and hardener, in an amount which results in a dyestuff concentration of 13 g./kg. of emulsion.

Solutions A to G are cast on a transparent film substrate, applying 3 g./m.<sup>2</sup> of silver. These cast films are exposed and processed as indicated in Example 1.

The results are summarized in the table below. The smaller value of the relative sensitivity log E represents higher sensitivity.

| Emulsion | Sensitization Maximum in nm | Color Development Relative Sensitivity log E |
|----------|-----------------------------|----------------------------------------------|
| A        | 620                         | 2.58                                         |
| B        | 600                         | 3.38                                         |
| C        | 640                         | 2.54                                         |
| D        | 660                         | 2.20                                         |
| E        | 660                         | 2.33                                         |
| F        | 560                         | weak image, cannot be evaluated              |
| G        | 560                         | 3.83                                         |

The sensitizers used according to the invention in emulsions A to E produce a higher sensitivity and result in a sensitization maximum which is displaced to longer wavelengths than in emulsions F and G, employed for comparison.

For a red-sensitive emulsion in a color reproduction material, sensitization with a maximum of 600 nm. and above is generally required, preferably at 640 to 700 nm.

#### EXAMPLE 6

Various ethanol solutions of sensitizers are added in each case to equal parts of a silver bromide-iodide emulsion containing 21 g. of silver, and 90 g. of gelatine per 1 kg. of emulsion, at 40° C., so that a sensitizer concentration of 150 mg./mol of silver results.

| Emulsion | Sensitizer of Formula |
|----------|-----------------------|
| A        | (66)                  |
| B        | (68)                  |
| C        | (70)                  |
| D        | (71)                  |

For comparison, emulsion E is also manufactured, containing a so-called symmetrical sensitizer of formula (XX), which differs from the sensitizers according to the invention.

Subsequently, an aqueous solution of the bluish-green dyestuff of formula (XXII) is added to emulsions A to E in addition to the usual additives, for example stabilizers, wetting agents, plasticizers and hardeners, in an amount which results in a dyestuff concentration of 4 g./kg. of emulsion.

Solutions A to E are cast on an opaque-white substrate, applying 1.8 g./m.<sup>2</sup> of silver. The exposure and processing of these cast films takes place as indicated in Example 5. The results are summarized in the table below.

| Emulsion | Sensitization Maximum in nm | Color Development Relative Sensitivity log E |
|----------|-----------------------------|----------------------------------------------|
| A        | 630                         | 3.30                                         |
| B        | 630                         | 3.22                                         |
| C        | 660                         | 3.07                                         |
| D        | 650                         | 3.22                                         |
| E        | 570                         | 4.02                                         |

The sensitizers used according to the invention in emulsions A to D produce a higher sensitivity and result in a sensitization maximum which is displaced to longer wavelengths than the sensitizer in emulsion E employed for comparison.

#### EXAMPLE 7

60 The procedure described in Example 6 is adopted. The compound of formula (68) is used as the sensitizer according to the invention. For comparison, emulsion B is manufactured, containing the so-called symmetrical sensitizer of formula (XX). The compound of formula (XXIII) is used as the bluish-green image dyestuff. The results are summarized in the table below.

| Emulsion | Sensitization Maximum in nm | Color Development Relative Sensitivity log E |
|----------|-----------------------------|----------------------------------------------|
| A        | 640                         | 3.54                                         |
| B        | 570                         | 3.83                                         |

75 The sensitizer used according to the invention in emulsion A

produces a higher sensitivity and results in a sensitization maximum which is displaced to longer wavelengths than the symmetrical sensitizer of emulsion B.

## EXAMPLE 8

The procedure described in Example 6 is adopted. The following are used as sensitizers according to the invention.

| Emulsion | Sensitizer of Formula |
|----------|-----------------------|
| A        | (66)                  |
| B        | (67)                  |
| C        | (68)                  |
| D        | (70)                  |
| E        | (71)                  |

For comparison, emulsions F and G are additionally manufactured, containing so-called symmetrical sensitizers which differ from the sensitizers according to the invention.

Emulsion F: Sensitizer of formula (XX)

Emulsion G: Sensitizer of formula (XXI)

The compound of formula (XXIV) is used as the bluish-green image dyestuff.

The results are summarized in the table below.

| Emulsion | Spectrum Maximum in nm |
|----------|------------------------|
| A        | 640                    |
| B        | 600                    |
| C        | 640                    |
| D        | 660                    |
| E        | 650                    |
| F        | 570                    |
| G        | 560                    |

The sensitizers used according to the invention in emulsions A to E result in a sensitization maximum which is displaced to longer wavelengths than the sensitizers employed for comparison purposes.

## EXAMPLE 9

The procedure described in Example 1 is adopted. The following are used as sensitizers according to the invention.

| Emulsion | Sensitizer of Formula |
|----------|-----------------------|
| A        | (16)                  |
| B        | (39)                  |
| C        | (40)                  |
| D        | (45)                  |
| E        | (51)                  |
| F        | (53)                  |
| G        | (56)                  |
| H        | (57)                  |
| I        | (83)                  |
| J        | (85)                  |

For comparison, emulsions K and L are additionally manufactured, containing so-called symmetrical sensitizers which differ from the sensitizers according to the invention.

Emulsion K: Sensitizer of formula (XXV)

Emulsion L: Sensitizer of formula (XXVI)



The results are summarized in the table below.

| Emulsion | Sensitizer | Spectrum Maximum in nm | Color Development Relative Sensitivity log E |
|----------|------------|------------------------|----------------------------------------------|
| 15       | A          | 655                    | 4.20                                         |
|          | B          | 655                    | 4.32                                         |
|          | C          | 650                    | 4.46                                         |
|          | D          | 660                    | 3.61                                         |
|          |            | 655                    | 4.01                                         |
|          | E          | 650                    | 4.28                                         |
|          | F          | 665                    | 4.01                                         |
|          | G          | 650                    | 4.26                                         |
|          | H          | 665                    | 3.92                                         |
|          | J          | 665                    | 3.55                                         |
| 25       | K          | 650                    | 5.55                                         |
|          | L          | 650                    | 4.52                                         |

The sensitizers used according to the invention in emulsions A to J produce a higher sensitivity and in part result in a sensitization maximum which is displaced to longer wavelengths than the sensitizers of emulsions K and L employed for comparison.

## EXAMPLE 10

The procedure described in Example 1 is adopted. The following are used as sensitizers.

| Emulsion | Sensitizer of Formula |                      |
|----------|-----------------------|----------------------|
| 40       | A                     | (16)                 |
|          | B                     | (39)                 |
|          | C                     | (40)                 |
|          | D                     | (45)                 |
|          | E                     | (51)                 |
|          | F                     | (53)                 |
|          | G                     | (55)                 |
|          | H                     | (56)                 |
|          | I                     | (57)                 |
|          | J                     | (83)                 |
| 50       | K                     | (85)                 |
|          | L                     | (XXV) for comparison |

The dyestuff of formula (XXIII) is used as the image dyestuff, and in particular so as to result in a dyestuff concentration of 24 g./kg. of emulsion.

The results are summarized in the table below.

| Emulsion | Sensitizer | Spectrum Maximum in nm | Color Development Relative Sensitivity log E |
|----------|------------|------------------------|----------------------------------------------|
| 60       | A          | 655                    | 3.32                                         |
|          | B          | 655                    | 3.61                                         |
|          | C          | 650                    | 3.72                                         |
|          | D          | 665                    | 3.27                                         |
|          | E          | 655                    | 3.28                                         |
|          | F          | 650                    | 3.55                                         |
|          | G          | 655                    | 3.62                                         |
|          | H          | 665                    | 3.23                                         |
|          | I          | 650                    | 4.04                                         |
|          | J          | 665                    | 3.03                                         |
| 70       | K          | 660                    | 3.04                                         |
|          | L          | 650                    | 5.45                                         |

The sensitizers employed according to the invention in emulsions A to K produce a higher sensitivity and in part result in a sensitization maximum which is displaced to longer wavelengths than the sensitizer of emulsion L employed for comparison.

**EXAMPLE 11**

The procedure described in Example 2 is adopted. The following are used as sensitizers according to the invention.

| Emulsion | Sensitizer of Formula |
|----------|-----------------------|
| A        | (16)                  |
| B        | (39)                  |
| C        | (40)                  |
| D        | (45)                  |
| E        | (51)                  |
| F        | (53)                  |
| G        | (55)                  |
| H        | (56)                  |
| I        | (57)                  |
| J        | (83)                  |
| K        | (85)                  |
| L        | (XXV) for comparison  |

The results are summarized in the table below.

| Emulsion | Spectrum      |                  | Color Development<br>Relative Sensitivity<br>log E |
|----------|---------------|------------------|----------------------------------------------------|
|          | Sensitization | Maximum<br>in nm |                                                    |
| A        |               | 650              | 2.77                                               |
| B        |               | 652              | 3.04                                               |
| C        |               | 645              | 2.83                                               |
| D        |               | 650              | 2.61                                               |
| E        |               | 650              | 2.79                                               |
| F        |               | 640              | 2.90                                               |
| G        |               | 650              | 3.52                                               |
| H        |               | 660              | 3.22                                               |
| I        |               | 645              | 2.97                                               |
| J        |               | 660              | 2.73                                               |
| K        |               | 660              | 2.38                                               |
| L        |               | 640              | 3.80                                               |

The sensitizers employed according to the invention in emulsion A to K produce a higher sensitivity and in part result in a sensitization maximum which is displaced to longer wavelengths than the sensitizer of emulsion L employed for comparison.

### EXAMPLE 12

The procedure described in Example 2 is adopted. The following are used as sensitizers.

| Emulsion | Sensitizer of Formula |
|----------|-----------------------|
| A        | (16)                  |
| B        | (39)                  |
| C        | (40)                  |
| D        | (45)                  |
| E        | (51)                  |
| F        | (55)                  |
| G        | (56)                  |
| H        | (57)                  |
| I        | (83)                  |
| J        | (85)                  |
| K        | (XXV) for comparison  |
| L        | (XXVI) for comparison |

The compound of formula (XXIII) is used as the bluish-green image dyestuff.

The results are summarized in the table below.

| Emulsion | Sensitization | Spectrum         | Color Development             |
|----------|---------------|------------------|-------------------------------|
|          |               | Maximum<br>in nm | Relative Sensitivity<br>log E |
| A        |               | 650              | 3.29                          |
| B        |               | 650              | 3.37                          |
| C        |               | 645              | 2.83                          |
| D        |               | 650              | 2.52                          |
| E        |               | 650              | 3.01                          |
| F        |               | 650              | 3.10                          |
| G        |               | 660              | 2.87                          |
| H        |               | 645              | 2.95                          |
| I        |               | 660              | 2.93                          |
| J        |               | 660              | 2.45                          |
| K        |               | 645              | 3.93                          |
| L        |               | 645              | 3.47                          |

20 The sensitizers used according to the invention in emulsions  
A to J produce a higher sensitivity and in part result in a sen-  
sitzation maximum which is displaced to longer wavelengths  
than the sensitizers of the emulsions K and L employed for  
25 comparison.

### 23 Comparison:

1. Photographic material for the silver dyestuff bleaching process which in at least one red-sensitive silver halide emulsion layer contains a bleachable azo dyestuff as the image 30 dyestuff, wherein this layer contains a red-sensitizer characterized by an absorption maximum above about 554 nm. and a sensitization maximum above about 625 nm. of the formula



in which A is a hydrogen atom or an alkyl group containing 1 to 4 carbon atoms; B<sub>1</sub> and B<sub>2</sub> each is a member selected from the group consisting of an alkyl radical containing 1 to 4 carbon atoms, an alkylcarboxylic acid radical containing 1 to 5 carbon atoms, a sulfatoalkyl radical containing 1 to 4 carbon atoms and an alkylsulfonic acid radical, wherein alkyl is a radical of the formula —C<sub>n</sub>H<sub>2n-1</sub>— and n is an integer of at most 4, provided that each of B<sub>1</sub> and B<sub>2</sub> is not simultaneously an acid group, R<sub>1</sub> and R<sub>2</sub> each is an aromatic ring system containing at most two six-membered rings which is fused-on in the manner indicated by the valency lines; Y<sup>-</sup> is an anion and Z is a sulfur or selenium atom.

55 2. Photographic material as claimed in claim 1, in which A is ethyl.



3. Photographic material as claimed in claim 1.



in which  $B_1$  is an ethyl, methylcarboxylic or ethylcarboxylic acid radical and  $B_2$  is ethyl.

4. Photographic material as claimed in claim 1, which con-

tains a red-sensitizer of formula



in which  $X_1$ ,  $X_2$ ,  $X_3$  and  $X_4$  each is a hydrogen atom, halogen atom, alkyl or alkoxy group which each contains 1 to 3 carbon atoms.

5. Photographic material as claimed in claim 4, which contains a red-sensitizer of formula



6. Photographic material as claimed in claim 5, in which  $X_1$ ,  $X_2$ ,  $X_3$  and  $X_4$  each is a hydrogen atom, a chlorine atom, a methyl, methoxy or ethoxy group.



in which  $X_1$ ,  $X_2$ ,  $X_3$  and  $X_4$  each is a hydrogen atom, a chlorine atom, a methyl, methoxy or ethoxy group.

7. Photographic material as claimed in claim 5, which contains a red-sensitizer of formula



50

55

60

65

70

8. Photographic material as claimed in claim 1, which contains a red-sensitizer of formula



9. Photographic material as claimed in claim 1, which contains a red-sensitizer of formula



10. Photographic material as claimed in claim 1, which contains a red-sensitizer of formula



11. Photographic material as claimed in claim 1, which contains a red-sensitizer of formula



75

PO-1050  
(5/69)

TEL-59/E

UNITED STATES PATENT OFFICE  
CERTIFICATE OF CORRECTION

Patent No. 3,647,466 Dated March 7, 1972

Inventor(s) HEINRICH BRUENGER ET AL

It is certified that error appears in the above-identified patent and that said Letters Patent are hereby corrected as shown below:

Column 18, line 53, "Y" should be --- Y  $\ominus$  ---.

Column 18, lines 57-64, delete the formula.

Column 18, lines 66-73, delete the formula.

Signed and sealed this 5th day of September 1972.

(SEAL)

Attest:

EDWARD M.FLETCHER, JR.  
Attesting Officer

ROBERT GOTTSCHALK  
Commissioner of Patents